

1

2,985,590

## LUBRICATING OIL COMPOSITIONS COMPRISING MERCAPTOBENZOTIAZOLE ESTER DERIVATIVES

Arnold J. Morway, Clark, and Jeffrey H. Bartlett, New Providence, N.J., assignors to Esso Research and Engineering Company, a corporation of Delaware

No Drawing. Original application Sept. 28, 1955, Ser. No. 537,304. Divided and this application Feb. 21, 1958, Ser. No. 716,531

6 Claims. (Cl. 252—47.5)

This invention relates to mercaptobenzothiazole carboxylic acid and ester derivatives thereof and compositions containing the same. More particularly, the invention relates to mercaptobenzothiazole low molecular weight carboxylic acid and high molecular weight ester derivatives. The compositions of the invention include lubricating oils, lubricating greases, gear oils, hydraulic fluids, cutting oils, etc.

This application is a division of our copending application Serial No. 537,304, filed September 28, 1955, and now abandoned.

Mercaptobenzothiazole is a well known vulcanizing accelerator useful in the preparation of rubber. Compounds of this type which contain a high percentage of sulfur in a non-corrosive form, would be a very desirable lubricant constituent, since it has been previously established that sulfur-containing compounds will enhance the load-carrying or extreme pressure characteristics of lubricants. Mercaptobenzothiazole is, however, substantially insoluble in mineral or synthetic lubricating oils. In accordance with the invention, it has now been found that certain mercaptobenzothiazole carboxylic acid and ester derivatives are soluble in oil, and that these sulfur- and nitrogen-containing compounds can be effectively utilized as lubricating oil and grease constituents. More particularly, it has been found that certain 2-mercaptopbenzothiazole acetic or propionic esters may be advantageously employed as extreme pressure additives in lubricating oil compositions. Furthermore, these ester compounds may be employed as the grease base or soap dispersant of lubricating grease compositions. In accordance with another aspect of this invention, it has been found that the acetic or propionic acid derivatives of 2-mercaptobenzothiazole can be employed as a constituent of a grease thickener, especially a metal soap-salt complex thickener.

The mercaptobenzothiazole compounds contemplated in this invention are represented by the following general structural formula



wherein  $n$  is an integer equal to 1 and 2, and R is selected from the group consisting of hydrogen and an aliphatic alkyl radical having from 8 to 20 carbon atoms. The alkyl group can be either straight or branched chain. Examples of the acid derivatives include:

2-mercaptobenzothiazole acetic acid

2-mercaptobenzothiazole propionic acid

The ester derivatives are exemplified by:

2-mercaptobenzothiazole acetic acid iso-octyl ester

2-mercaptobenzothiazole acetic acid  $C_8$  Oxo ester

2-mercaptobenzothiazole acetic acid nonyl ester

2-mercaptobenzothiazole acetic acid dodecyl ester

2

- 2-mercaptobenzothiazole acetic acid tridecyl ester  
 2-mercaptobenzothiazole acetic acid isotridecyl ester  
 2-mercaptobenzothiazole acetic acid  $C_{13}$  Oxo ester  
 2-mercaptobenzothiazole acetic acid tetradearyl ester  
 2-mercaptobenzothiazole acetic acid hexadecyl ester  
 2-mercaptobenzothiazole acetic acid octadecyl ester  
 2-mercaptobenzothiazole acetic acid arachidyl ester

In order to avoid unnecessary duplication the 2-mercaptobenzothiazole propionic acid esters are not listed, but they correspond exactly to the compounds described above with the exception that the carboxylic acid portion of the compounds is a propionic acid instead of an acetic acid radical.

In general, the mercaptobenzothiazole carboxylic acid derivatives are prepared from 2-mercaptobenzothiazole according to the following steps:



wherein X is a halogen selected from the group consisting of chlorine, bromine and iodine, and  $n$  is an integer equal to 1 and 2. Examples of the monohalogenated carboxylic acids include: monochloroacetic acid, monobromoacetic acid, monoiodoacetic acid, monochloropropionic acid, monobromopropionic acid, and monoiodopropionic acid. Potassium hydroxides may be used in place of sodium hydroxide or sodium alkoxide in the preparation of the alkali metal salt of mercaptobenzothiazole.

Temperatures within the range of about 0 to 50°C. are employed in preparing the alkali metal salt of mercaptobenzothiazole. The alkali metal salt of mercaptobenzothiazole is then reacted with the alkali metal salt of monohalogenated acetic or propionic acid, for example, at temperatures in the range of about 0 to 75°C.

The preparation of ester derivatives of mercaptobenzothiazole acetic and propionic acids can be readily accomplished by reacting the alkali metal salt of mercaptobenzothiazole with esters of the monohalogenated substituted acetic and propionic acids at temperatures within the range of about 0 to 75°C. The esters of the monohalogenated substituted acetic and propionic acids correspond to the following general formula:



where X is a halogen selected from the group consisting of chlorine, bromine and iodine,  $n$  is an integer from 1 to 2, and R is a straight or branched chain aliphatic alkyl radical containing from 8 to 20 carbon atoms, which is derived from the corresponding alcohol. The above esters are prepared by esterifying the corresponding monohalogenated substituted carboxylic acids with an alcohol having the desired number of carbon atoms. Alcohols contemplated in this invention included:

Octyl alcohol  
 Iso-octyl alcohol  
 $C_8$  Oxo alcohol  
 Nonyl alcohol  
 Decyl alcohol

Isododecyl alcohol  
 Tridecyl alcohol  
 Isotridecyl alcohol  
 $C_{13}$  Oxo alcohol  
 Tetradecyl alcohol

Isodecyl alcohol  
Dodecyl alcohol

Hexadecyl alcohol  
Octadecyl alcohol, etc.

It will be noted that branched chain as well as straight chain aliphatic alcohols may be employed in preparing the ester derivatives of mercaptobenzothiazole. The Oxo alcohols described above are prepared by catalytically hydrogenating the aldehydes prepared in the well known Oxo process, which involves the carbonylation of olefins with carbon monoxide and hydrogen in the presence of a cobalt catalyst at a temperature of about 300° to 400° F. and a pressure of about 2500 to 4000 p.s.i.g. The mono-olefinic carbonylation feed can comprise C<sub>7</sub> to C<sub>19</sub> olefins derived from cracked gases, from Fischer-Tropsch products or from polymers of ethylene or propylene. The Oxo process as well as the preparation of Oxo alcohols are described in detail in U.S. Patent No. 2,593,428, issued April 27, 1952, to Fischer, Knoth and Newberg. The Oxo alcohols contemplated in this invention are branched chain saturated aliphatic alcohols.

The ester derivatives may also be prepared by esterifying the 2-mercaptobenzothiazole acetic or propionic acid, prepared as described above, directly with one of the alcohols, listed above. This method is illustrated as follows:



wherein *n* is an integer equal to 1 or 2 and R is a straight or branched chain aliphatic radical containing from 8 to 20 carbon atoms.

In the following example the preferred method of preparing the ester derivatives of 2-mercaptobenzothiazole is described.

#### EXAMPLE I

##### A. Preparation of mercaptobenzothiazole acetic acid

A 3 liter 3 necked flask equipped with a stirrer and thermometer was charged with 285 g. of chloroacetic acid and 700 cc. methanol. This mixture was cooled to 0° C. and then treated with 163 g. of sodium methoxide dissolved in 500 cc. methanol, thus yielding the sodium chloroacetate.

A 5 liter 4 necked flask was also set up and was equipped with a stirrer, condenser, thermometer and dropping funnel. It was then charged with 501 g. (3 m.) mercaptobenzothiazole and 800 cc. methanol. To this mixture was added 162 g. sodium methoxide dissolved in 500 cc. methanol. The resulting mixture was cooled to 0° C. and then the sodium chloroacetate solution was added through the dropping funnel over a period of about 10 minutes. Heat was applied and gradually raised to 68° C. during 1½ hours. Then the product was transferred to a 12 liter flask where it was dispersed in water and acidified with HCl followed by 3 water washes. The washed product was dissolved in a mixture of benzol and methyl ethyl ketone, dried with Na<sub>2</sub>SO<sub>4</sub>, filtered and evaporated on a steam bath leaving a solid residue of 562 g. of 2-mercaptobenzothiazole acetic acid. Acid No.=0.403 ceq./gm.

##### B. Preparation of the C<sub>13</sub> Oxo ester of mercaptobenzothiazole acetic acid

A 2 liter 3 necked flask equipped with a stirrer, thermometer and a water trap with a condenser was charged with:

Mercaptobenzothiazole acetic acid ----- g. 113  
C<sub>13</sub> Oxo alcohol ----- g. 200 75

Toluene sulfonic acid ----- g. 1  
Toluene ----- cc. 400

The above mixture was refluxed for 3½ hours at 120-125° C. during which time 15 cc. of water was collected in the trap. The resulting product was diluted with 500 cc. toluene and given 3 washes with 5% NaOH followed by 3 water washes, then evaporated on the steam bath for removal of the toluene.

The residue was stripped in a short path still to a pot temperature of 210° C. at 0.5 mm. leaving 175 g. of bottoms. This was treated with 15 g. of Super Filtral clay at 150° C. for 5 minutes and filtered through Hyflo<sup>1</sup> leaving a finished ester with the following analysis:

Acid No.=0.010 ceq./gm.  
Ester No.=0.266 ceq./gm.

##### 20 C. Preparation of isoctyl ester of mercaptobenzothiazole acetic acid

A 3 liter 4 necked flask equipped with a stirrer, condenser, thermometer and dropping funnel was charged with 334 g. mercaptobenzothiazole and 600 cc. methanol. To this mixture was added 110 g. sodium methoxide dissolved in 500 cc. methanol. The resulting mixture was cooled to 10° C. when 413 g. of isoctyl ester of chloroacetic acid was added during 2 minutes. Heat was then applied and the temperature raised to 70° C. during 45 minutes. After cooling to 55° C. the mixture was filtered through Hyflo. The methanol was then evaporated, and the residue distilled in a short path still. A fraction of 274 g. was obtained at 155° to 185° C. at 0.7 mm. with most of it boiling at 175° C. There was a remaining residue of 56 g.

As noted above, the 2-mercaptobenzothiazole aliphatic esters of the invention can be effectively utilized as load carrying or extreme pressure additives in lubricating oils. Mineral lubricating oils are the preferred menstrua, and they may be any of the well known mineral lubricating oils with which the art is familiar. Petroleum distillates from either naphthenic or paraffinic base stocks having a viscosity from about 35 to 250 SUS at 210° F. may be used as well as mixtures of the same; the choice of base oil depending upon the lubricating service contemplated. Synthetic lubricating oils may also be used as the vehicles such as hydrocarbon, hydrocarbon polymer, ester, complex ester, formal, mercaptal, polyalkylene oxide, silicone or similar types. More particularly, synthetic oils such as di-2-ethylhexyl sebacate, di-C<sub>8</sub> Oxo azelate, and other branched chain simple esters of dicarboxylic acids as well as complex esters prepared from glycols, dicarboxylic acids and alcohols and/or monocarboxylic acids. Mixtures of mineral and synthetic oils may also be employed. For special applications, animal, vegetable or fish oils, or their hydrogenated or voltolized products may be employed, either alone or in admixture with mineral oils. The amount of the mercaptobenzothiazole carboxylic acid ester additive used in the lubricating oil will ordinarily be from about 3 to 15 wt. percent, preferably about 5 to 10 wt. percent, based on the total weight of the compositions.

#### EXAMPLE II

A number of lubricating oil compositions were prepared comprising a mineral lubricating oil having a viscosity of 55 SUS/210° F. and minor amount of 2-mercaptobenzothiazole acetic acid C<sub>13</sub> Oxo and C<sub>8</sub> Oxo esters. The C<sub>8</sub> Oxo ester of 2-mercaptobenzothiazole was not completely soluble, nevertheless it showed effective extreme pressure

<sup>1</sup> Diatomaceous earth.

additive properties. The composition and properties of the lubricating oils tested are tabulated below:

TABLE I

| Composition                                                                                                                        | Almen Test      |               |
|------------------------------------------------------------------------------------------------------------------------------------|-----------------|---------------|
|                                                                                                                                    | Weights Carried | Pin Condition |
| (A) Mineral lubricating oil (55 SUS @ 210° F.)                                                                                     | 2               | Sheared.      |
| (B) Mineral lubricating oil (55 SUS @ 210° F.) + 5 wt. percent of 2-mercaptopbenzothiazole acetic acid C <sub>13</sub> Oxo ester.  | 15              | Excellent.    |
| (C) Mineral lubricating oil (55 SUS @ 210° F.) + 10 wt. percent of 2-mercaptopbenzothiazole acetic acid C <sub>13</sub> Oxo ester. | 15              | Do.           |
| (D) Mineral lubricating oil (55 SUS @ 210° F.) + 10 wt. percent of 2-mercaptopbenzothiazole acetic acid C <sub>8</sub> Oxo ester.  | 15              | Do.           |

It will be noted from the above data that the esters of the invention are valuable as lubricating oil additives for enhancing the load-carrying or extreme pressure characteristics.

In accordance with another aspect of the invention, the 2-mercaptopbenzothiazole carboxylic acid esters of the invention can also be employed as grease bases or as the dispersants for metal soap, metal soap-salt complex or metal mixed salt complex grease thickeners. Non-soap grease thickeners such as silica gel, hydrocarbon polymers, etc., may also be used. When employed as the grease base the esters of the invention will ordinarily be used in amounts within the range of about 50 to 95 wt. percent, preferably about 60 to 90 wt. percent, based on the total weight of the grease composition. It is also contemplated that any of the conventional grease additives such as oxidation inhibitors, pour depressants, corrosion inhibitors and the like can be incorporated in the grease compositions described above.

The following example is illustrative of grease compositions prepared in accordance with this feature of the invention.

## EXAMPLE III

A lubricating grease was prepared from the following ingredients:

| Formulation                                                         | Percent Weight |
|---------------------------------------------------------------------|----------------|
| Glacial acetic acid.....                                            | 12.0           |
| Commercial capric acid.....                                         | 6.0            |
| Hydrated lime.....                                                  | 9.8            |
| Phenyl alpha-naphthylamine.....                                     | 1.0            |
| 2-mercaptopbenzothiazole acetic acid C <sub>13</sub> Oxo ester..... | 71.2           |
| Percent                                                             |                |
| 1 Caprylic acid.....                                                | 24.1           |
| 2 Capric acid.....                                                  | 57.5           |
| 3 Lauric acid.....                                                  | 17.8           |

*Preparation.*—The hydrated lime and 2-mercaptopbenzothiazole acetic acid C<sub>13</sub> Oxo ester were charged to a steam heated grease kettle with mixing. Without the addition of external heating the acetic acid and the capric acid were charged with mixing to the slurry of lime in the ester. The temperature rose to about 165° F. After about one-half hour the temperature was about 120° F., and the grease mixture heated to about 320° F. for about one hour to effect dehydration. Phenyl alpha-naphthylamine was then added, and the grease mixture cooled to about 180° F. by passing cold water through the kettle jacket. The resulting grease composition was then Gaulin homogenized at 6000 p.s.i.

## Properties:

|                              |                             |
|------------------------------|-----------------------------|
| Appearance                   | Excellent, smooth, uniform. |
| Dropping point, ° F.         | 500+.                       |
| Penetrations (77° F. mm./10) |                             |
| Unworked                     | 275.                        |
| Worked (60 strokes)          | 295.                        |
| Worked (100,000 strokes)     | 340.                        |

|                                                         |        |
|---------------------------------------------------------|--------|
| Norma-Hoffman oxidation test<br>(hrs. to 5 p.s.i. drop) | 350.   |
| Lubrication life, hours (250° F.,<br>10,000 r.p.m.)     | 1700+. |
| Extreme pressure properties,<br>Timken test (45 lbs.)   | Pass.  |
| Shell four ball test (extreme pres-<br>sure index)      | 50.3.  |

10 Other conventional grease thickeners, both soap and non-soap types, may be employed in place of the mixed metal salt complex described in Example III when the ester derivatives of 2-mercaptopbenzothiazole of the invention are utilized as grease bases. For example, any of the commonly known grease-making soaps such as the metal soaps of high molecular weight saturated or unsaturated carboxylic acids having from 12 to 30 carbon atoms per molecule, preferably about 16 to 22 carbon atoms, may be utilized. Operable metals include the alkali metals; sodium, lithium and potassium; and the alkaline earth metals: calcium, barium, strontium and magnesium. The high molecular weight fatty acids are exemplified by lauric acid, myristic acid, palmitic acid, stearic acid, hydroxy stearic acid, oleic acid, hydrogenated fish oil acids, linoleic acid, arachidic acid, behenic acid, etc. Glycerides of the above acids, vegetable fat, tallow, etc. may also be employed as the saponifiable material.

15 Suitable complex thickening agents include:

(a) The soap-salt complexes prepared from the metal salts of low molecular weight carboxylic acids having from 1 to 3 carbon atoms per molecule, and metal soaps of high molecular weight carboxylic acids having from 12 to 30 carbon atoms per molecule, wherein the mol ratio of the low to high molecular weight acids is about 1:1 to 40:1, preferably about 8:1 to 25:1.

(b) The mixed salt complexes, as described above in Example III, prepared from the metal salts of low molecular weight carboxylic acids having from 1 to 3 carbon atoms per molecule, and metal salts of intermediate molecular weight carboxylic acids having from 7 to 10 carbon atoms per molecule, wherein the mol ratio of low to intermediate molecular weight acids is about 2:1 to 40:1, preferably about 4:1 to 25:1.

(c) The soap-salt complexes prepared from a metal salt of acetic acid, metal salts of medium molecular weight carboxylic acids having from 3 to 10 carbon atoms per molecule and metal soaps of high molecular weight carboxylic acids having from 12 to 30 carbon atoms per molecule; wherein the mol ratio of acetic acid to the medium and high molecular weight acids is about 0.5:1 to 10:1, and the difference in number of carbon atoms per molecule between the high and medium molecular weight carboxylic acids is at least 7, preferably about 7 to 15.

55 The high molecular weight carboxylic acids useful for preparing the complex thickeners described above are the well known saturated and unsaturated, grease-making fatty acids which were previously described with respect to the preparation of the conventional metal soap grease thickeners.

60 The intermediate molecular weight acids are those aliphatic monocarboxylic acids containing from about 7 to 10 carbon atoms, preferably about 8 or 9 carbon atoms, per molecule. Either saturated or unsaturated fatty acids may be utilized, although the saturated fatty acids are preferred. Suitable acids include: 5-methyl-2-hexanoic, heptanoic, octanoic, 2-ethyl-hexanoic, C<sub>8</sub> Oxo, nonanoic, decanoic, C<sub>10</sub> Oxo acids, etc.

65 The medium molecular weight carboxylic acids include straight and branched chain saturated aliphatic carboxylic acids, hydroxy aliphatic mono- and poly-carboxylic acids, aromatic mono- and poly-carboxylic acids and anhydrides thereof, and heterocyclic acids containing from about 3 to 10, preferably about 6 to 9, carbon atoms per molecule. Suitable acids include: pentanoic,

hexanoic, heptanoic, octanoic, nonanoic, decanoic, isobutyric,  $C_5$  Oxo,  $C_8$  Oxo,  $C_9$  Oxo,  $C_{10}$  Oxo, glyceric, benzoic, hydroxy benzoic, toluic, o-phthalic, phthalic anhydride, terephthalic, furoic, thiophene carboxylic, etc.

The low molecular weight carboxylic acids capable of being used in the preparation of the complex thickeners include saturated and unsaturated carboxylic acids having from about 1 to 3 carbon atoms per molecule, such as formic, acetic, acrylic and similar acids including their hydroxy derivatives, e.g. lactic acid. Mono-carboxylic acids are particularly useful, and acetic acid is especially preferred.

The alkaline earth metals such as calcium, barium and strontium are particularly useful for preparing the complex grease thickeners. Calcium is especially preferred. The alkali metals such as sodium, potassium and lithium can also be employed, though they are not as effective for the preparation of these complex thickeners as the alkaline earth metals. Magnesium and zinc can also be used for this purpose.

In general, the amount of metal soap or complex grease thickener in the 2-mercaptopbenzothiazole carboxylic acid ester base greases of the invention will vary from about 2 to 20 wt. percent, preferably from about 4 to 15 wt. percent; the percentages being based on the weight of the total composition.

In accordance with another feature of this invention, the low molecular weight carboxylic acid derivatives of 2-mercaptopbenzothiazole are useful in the preparation of the metal complex grease thickeners described above. The carboxylic acid derivatives contemplated in this aspect of the invention correspond to the following structural formula:



wherein  $n$  is an integer equal to 1 and 2. More particularly, it has now been found that 2-mercaptopbenzothiazole acetic and propionic acids can be effectively utilized in the preparation of metal soap-salt complex grease thickeners.

#### EXAMPLE IV

A lubricating grease composition was prepared from the following ingredients:

| Formulation                                                      | Percent Weight |
|------------------------------------------------------------------|----------------|
| Glacial acetic acid                                              | 12.0           |
| 2-Mercaptopbenzothiazole acetic acid                             | 3.0            |
| Stearic acid                                                     | 3.0            |
| Hydrated lime                                                    | 9.0            |
| Phenyl alpha naphthylamine                                       | 0.5            |
| Mineral lubricating oil (65 SUS @ 210° F.)                       | 72.5           |
| Mol ratio (acetic to higher acids)                               | 5:1            |
| Mol ratio (2-mercaptopbenzothiazole acetic acid to stearic acid) | 0.5:1          |

*Preparation.*—The mineral lubricating oil, the lime, stearic acid and 2-mercaptopbenzothiazole acetic acid were charged to a fire heated grease kettle with stirring to form a slurry. The slurry was warmed to 140° F., the acetic acid added, and the heating continued to a temperature of about 500° F. The heating was then discontinued, and the grease mixture was cooled to 200° F. while agitating. At this point, phenyl alpha naphthylamine was added, and the grease mixture was Gaulin homogenized at 6000 p.s.i.

#### Properties:

|                                        |                             |
|----------------------------------------|-----------------------------|
| Appearance                             | Excellent, smooth, uniform. |
| Percent free alkalinity (percent NaOH) | 0.76.                       |
| Dropping point, ° F.                   | 500+.                       |

#### Penetration (77° F. mm./10)—

|                          |      |
|--------------------------|------|
| Unworked                 | 300. |
| Worked (60 strokes)      | 310. |
| Worked (100,000 strokes) | 355. |

Phase change up to 400° F. None.

Norma-Hoffman oxidation test (hrs. to 5 p.s.i. drop) 350.

Lubrication life, hours (10,000 r.p.m., 250° F.) 1034.1

E.P. properties, Almen shock load 15 wghts., excellent pin condition.

Timken test (45 lbs.) Pass.

<sup>1</sup> Discontinued test. Inspection of bearings and grease showed them to be in good condition.

The calcium soap-salt complex thickener of the above example is similar to the complex thickener type (c) described above, with the exception that 2-mercaptopbenzothiazole acetic acid is employed as the medium molecular weight carboxylic acid. The metals, the low molecular weight carboxylic acids and the high molecular weight carboxylic acids described above in connection with type (c) are also applicable for preparing the metal soap-salt complex thickeners of this invention.

Mineral or synthetic lubricating oils described above with respect to the lubricating oil composition of the invention can also be utilized as the grease base for this feature of the invention. Ordinarily about 2 to 40 wt. percent, preferably about 5 to 30 wt. percent, of the complex grease thickener is employed with from about 60 to 98 wt. percent, preferably about 70 to 90 wt. percent, of the oleaginous vehicle.

In brief summary, the invention pertains to 2-mercaptopbenzothiazole acetic or propionic acids and ester derivatives thereof, corresponding to the following structural formula:



wherein  $n$  is an integer equal to 1 and 2, and R is selected from the group consisting of hydrogen and a straight or branched chain, aliphatic alkyl radical having from 8 to 20 carbon atoms. The ester derivatives of the invention can be utilized as lubricating oil additives in amounts of about 3 to 15 wt. percent to contribute extreme pressure properties to the final lubricating oil composition. These ester derivatives may also be effectively utilized in amounts ranging from about 50 to 95 wt. percent as grease bases or soap dispersants in the preparation of lubricating grease compositions having long lubrication lives and excellent extreme pressure characteristics as well as other desirable grease properties.

It is also within the scope of the present invention to employ the acetic and propionic acid derivatives of 2-mercaptopbenzothiazole themselves as constituents in the preparation of metal soap-salt complex grease thickeners.

The invention is not limited to the specific materials and conditions of the foregoing examples. These materials and conditions may be varied within the limits indicated in the general portions of the specification. Though the acetic and propionic acid and ester derivatives of 2-mercaptopbenzothiazole are the preferred compounds of the invention, the invention is necessarily limited to these particular acid or ester derivatives. Nevertheless, it has been found that the most desirable acid and ester derivatives are those in which the carboxyl group has a relatively close proximity to the 2-mercaptop sulfur atom.

It is also contemplated that the lubricating compositions of the invention can contain any of the conventional additives such as oxidation inhibiting pour depressants, corrosion inhibitors and the like.

What is claimed is:

1. A lubricating oil composition comprising a major amount of a lubricating oil and a minor but load carrying

improved amount of a compound having a structure corresponding to the following formula



wherein  $n$  is an integer equal to 1 and 2, and R is an alkyl radical containing from 8 to 20 carbon atoms.

2. The lubricating oil composition of claim 1 wherein the amount of said compound is from 3 to 15% by weight, based on the weight of the total composition.

3. The lubricating oil composition of claim 1 wherein said compound is 2-mercaptopbenzothiazole acetic acid C<sub>13</sub> branched chain alkyl ester.

4. The lubricating oil composition of claim 1 wherein R is an iso-octyl radical.

5. A mineral lubricating oil composition comprising a major amount of mineral lubricating oil and about 3 to 15 wt. percent, based on the weight of the total composition, of a compound having a structure corresponding to the following formula



wherein  $n$  is an integer equal to 1 and 2, and R is an alkyl radical containing from 8 to 20 carbon atoms.

6. A method for lubricating metal surfaces subjected to extreme pressure which comprises maintaining on said surfaces a lubricating oil containing a load carrying improving amount of a compound having the following formula



wherein  $n$  is an integer equal to 1 and 2, and R is an alkyl radical containing from 8 to 20 carbon atoms.

References Cited in the file of this patent

UNITED STATES PATENTS

|    |           |                |               |
|----|-----------|----------------|---------------|
| 20 | 2,725,382 | Harmon         | Nov. 29, 1955 |
|    | 2,734,869 | Mullen et al.  | Feb. 14, 1956 |
|    | 2,796,404 | Levin          | June 18, 1957 |
|    | 2,799,656 | Mikeska et al. | July 16, 1957 |
|    | 2,801,969 | Morway et al.  | Aug. 6, 1957  |
| 25 | 2,841,556 | Swenson et al. | July 1, 1958  |
|    | 2,844,536 | Morway         | July 22, 1958 |